

April 13, 1937.

H. G. KITTREDGE ET AL

2,077,112

IMITATION LEATHER PAPER

Filed Dec. 28, 1934

FIG. 1.



INVENTORS  
HARVEY G. KITTREDGE &  
ALBERT J. TURNER

BY *John W. Dill*  
ATTORNEYS

## UNITED STATES PATENT OFFICE

2,077,112

## IMITATION LEATHER PAPER

Harvey G. Kittredge and Albert J. Turner, Dayton, Ohio, assignors to The Kay and Ess Chemical Corporation, Dayton, Ohio, a corporation of Delaware

Application December 28, 1934, Serial No. 759,550

1 Claim. (Cl. 91—70)

This invention relates to a new article of manufacture for use as imitation leather having the appearance, feel and body of leather.

It is the object of the invention to provide imitation leather paper which has a wrinkled, leather-like surface but which is not embossed, pressed or formed.

It is an object to provide such a leather-like paper, paper board or any other cellulose material which has such an appearance.

It is a further object to provide such an imitation leather paper that the leather finish will be on one side but the other side will remain in its normal condition for ordinary uses of packaging, printing, etc.

It is an object to provide a product to which the leather-like surface can be applied in any color, which can be applied and dried at ordinary temperatures of a room from sixty to seventy degrees Fahrenheit, or which may be baked as high as two hundred and twenty five degrees Fahrenheit; it is a further object to provide such a leather-like paper consisting of the wrinkled leather-like coating that can be sprayed, dipped, impregnated or applied in any manner to the surfaces of the paper without the necessity of any intermediate backing, sizing or other treatment of the paper.

It is an object to provide such a leather-like finish that will penetrate the surface of the paper sufficiently to form an intimate bond with the paper or other cellulose material to which it is applied but which will not penetrate the paper itself completely.

It will be understood in this application that when we refer to paper, we refer to any compound of cellulose.

Referring to the drawing:

The figure is a section through a cellulose backing, such as of paper, with the imitation leather finish mounted thereon.

Referring to the drawing in detail, 1 is a cellulose backing of paper, pasteboard, straw-board, cellophane, or any other cellulose material. 2 indicates the zone of penetration forming the bond between the paper 1 and the imitation leather finish 3. This finish is corrugated in substantially regular corrugations indicated at 4.

Upon the application of this finish, depending upon its exact composition, the finish will begin to wrinkle and will be completely wrinkled substantially throughout the body of the finish.

Even though the paper or other supporting backing is of very thin material, its wrinkle will not be imparted through the material. The

paper is opaque and the imitation leather finish will not penetrate through or be seen from the reverse side of the paper.

It is therefore possible to either have the plain paper on the opposite side from the finish for printing and the like, or a finish of the same or different color can be imparted to the supporting medium 1.

In applying this imitation leather finish, as hereinafter described, it is essential that the temperature of drying be not carried to a point where the paper will be injured. It is possible with our invention to keep within the limits of safety for the paper as the finishes which we provide range from those that dry in the air at room temperatures from 60 to 70 degrees Fahrenheit to those that can be baked at from 200 to 225 degrees Fahrenheit.

Typical compounds for the production of this new article of manufacture are as follows:

## EXAMPLE 1

In this example we use one of two varnishes, or a combination of two varnishes with a drier. These varnishes are designated Varnish "A" and Varnish "B".

## Varnish A

A typical formula is the following:

|                             | Pounds | 30 |
|-----------------------------|--------|----|
| Amberol B/S 1 Lt            | 67     |    |
| Litharge                    | 3 1/2  |    |
| Manganese linoleate (solid) | 8 1/2  |    |
| Cobalt linoleate (solid)    | 2      |    |
|                             |        | 35 |
| China-wood oil              | 20     |    |
| Linseed oil                 | 2 1/4  |    |
| Heavy petroleum naphtha     | 14     |    |
| Light petroleum naphtha     | 14     | 40 |

Amberol is a phenol, formaldehyde, synthetic resin. It is made as follows: to one hundred parts of phenol aldehyde resin difficultly fusible and only partly soluble in benzol and other solvents and produced, for instance, by heating 108 parts of cresol with 60 to 75 parts of formaldehyde (30% by weight) and distilling off the water and the uncombined cresol, are added gradually to 800 parts of melted colophony. The whole mixture is then heated in an autoclave until a resin is produced which is clear in the cold, homogeneous and free from smell of phenol. The volatile substances are then removed while stirring and 100 parts of glycerol of 28 degrees Bé. are added in small quantities whereupon the

mixture is heated to 250 degrees C. and kept at this temperature for several hours while being stirred carefully. A typical formula for amberol is shown in United States Patent No. 1,623,901.

In order to prepare this varnish, we first take 20 gallons of China wood oil or tung oil and 2 1/4 gallons refined linseed oil. These oils are mixed and heated at a normal rate to 480 degrees F. They are then pulled from the fire. These oils may undergo an automatic rise in temperature thereafter beyond 480 degrees F., but this is unnecessary and too great a rise should be avoided.

When the temperature of these oils has started to drop reaching approximately 475 degrees F., we add 3 1/2 pounds of litharge, stirring until the litharge is taken up by the oil. The temperature of this batch is then run back and forth between 460 degrees and 470 degrees, being held within this range for approximately 30 minutes and in some cases a little longer until sufficient body has been imparted to the oil and litharge.

Thereafter we add 8 1/2 pounds of manganese solid linoleate and 2 pounds of cobalt solid linoleate. These soluble driers melt into the batch.

We then add 67 pounds of synthetic resin solid, known to the trade as "Amberol B/S 1 Light." This is melted at a low heat. Then the temperature is carried back to approximately 425 degrees F.

We then thin the batch at once with 14 gallons each of heavy and light petroleum naphtha.

The resulting compound may be used by itself or in combination with the product of the formula hereinafter recited.

Thereafter we prepare Varnish B.

#### Varnish B

This formula is as follows:

|                         | Pounds  |
|-------------------------|---------|
| South Sea gum (Batu)    | 67      |
| Litharge                | 3 1/2   |
| Manganese linoleate     | 8 1/2   |
| Cobalt linoleate        | 2       |
|                         | Gallons |
| China-wood oil          | 20      |
| Linseed oil             | 2 1/4   |
| Heavy petroleum naphtha | 20      |
| Light petroleum naphtha | 20      |

The cooking is carried out in this manner. Sixty-seven pounds of South Sea gum, also known as Batu gum, are run in the ordinary approved fashion customary in varnish making. Then 20 gallons of China-wood oil and 2 1/4 gallons of refined linseed oil are mixed and heated slowly until they reach 300 or 350 degrees F., when they are added slowly to the gum when the latter has been well run.

The mixture is then carried to a temperature of 460 to 470 degrees F. and held within this range, in order to impart body to the mixture, for about 30 minutes or a little longer.

We then stir into the batch 3 1/2 pounds of litharge until it is taken up and fully incorporated in the batch. The 8 1/2 pounds of manganese solid linoleate and 2 pounds of cobalt solid linoleate are allowed to melt in the batch.

We then thin at once with 20 gallons each of heavy and light petroleum naphtha. Turpentine may be substituted for the naphtha.

In order to make the compound of this invention, either one of the above varnishes or both are combined with raw tung (China-wood) oil and a drier. A thinner can be added optionally.

The proportion of Varnish A with respect to Varnish B may be two to one, or vary therebetween, or Varnish B with respect to Varnish A may be two to one, or vary therebetween. In either event, the China-wood oil will vary in number of parts from approximately 5 to 25 parts. The drier will vary from approximately 5 to 25 parts, and the thinner will vary from 1 to 10 parts, depending upon the viscosity desired.

A typical example of a satisfactory compound for the practice of this invention is the following:

|                           | Parts  |
|---------------------------|--------|
| Varnish A                 | 81     |
| Varnish B                 | 40 1/2 |
| Raw tung (China-wood oil) | 9      |
| Drier                     | 9      |
| Petroleum naphtha         | 5-10   |

To one gallon of this compound we add 5 to 7 pounds of the desired color, previously ground in spar varnish.

Varnish A has the function of fast drying, and imparts a high luster. Varnish B has a medium drying rate, and provides a low luster. China-wood oil facilitates a very wrinkled drying with out gloss and adds opacity to the product. The thinner controls the viscosity and the drier has the following functions and characteristics.

When the compound of this invention is applied it must first flow out evenly on the surface treated and then the drying must begin almost at once on the surface of the wet compound by the formation of microscopic wrinkles. This initial wrinkling then proceeds through the whole thickness of the film as the complete drying proceeds.

The preferred drier that we have found to best serve this purpose comprises linoleate of lead, linoleate of cobalt, and linoleate of manganese. The cobalt and manganese, particularly the cobalt, accelerate the surface drying, as described above, while the lead and manganese are utilized for completing the drying completely through the film. This combination of cobalt and manganese supplies quick initial surface drying necessary, while the lead and the manganese supply the necessary catalytic action for the drying through the film.

#### Drier example

One of the preferred formulas which we have used is as follows:

|                        | Pounds |
|------------------------|--------|
| Linoleate of lead      | 385    |
| Linoleate of cobalt    | 889    |
| Linoleate of manganese | 14     |

These are melted at as low heat as possible, and when entirely fluid the mass is thinned with 1202 gallons of turpentine, either gum spirits or wood spirits, or some slowly evaporating coal tar fraction, such as xylene. It will be understood that the proportions of these elements of the drier can be varied according to the result desired. By adjusting these proportions the velocity of the surface drying and drying throughout the film can be regulated.

#### EXAMPLE 2

When it is desired particularly to utilize light colors and pastel shades in the imitation leather finish which may be baked at lower temperature with the minimum of discoloration, the finish of the present example is employed provided the temperature is not taken beyond approximately 225 degrees F. so as not to injure the paper.

In this example there are two varnishes known as Varnish C and Varnish D. Either one or both varnishes may be employed.

*Varnish C*

5 In order to make the first varnish designated as above, we take 100 pounds of Amberol B/S 1 Lt. and 14 gallons of raw China-wood oil, heating the China-wood oil and the above synthetic resin in a varnish kettle to 550 degrees F. Three pounds of linoleate of lead and one pound of linoleate of cobalt are then added and stirred thoroughly. The batch is then allowed to cool to 450 degrees F. and then reduced with 32 gallons of petroleum naphtha.

*Varnish D*

20 In order to make this varnish we take 200 pounds of a pure phenolic resin made by condensing phenol, a phenol derivative and formaldehyde and twenty gallons of raw China-wood oil. We place these in a varnish kettle raising the temperature slowly in about twenty-five minutes to 450 degrees F. We hold at this temperature for twenty minutes. We then thin with 20 gallons of toluol and 60 gallons of petroleum naphtha.

25 A typical varnish or enamel for making a white imitation leather finish is made up as follows:

|                                                                       |         |        |
|-----------------------------------------------------------------------|---------|--------|
| 30 Varnish C                                                          | gallons | 11 1/4 |
| Varnish D                                                             | do      | 6 3/4  |
| Raw China-wood oil                                                    | do      | 1 3/4  |
| Thinner composed of equal parts of toluol<br>35 and petroleum naphtha | gallons | 1-2    |
| Paste composed of pure titanium dioxide<br>ground in a spar varnish   | pounds  | 120    |

40 This enamel may be applied in any manner, as by inking rolls or by spray. When the supporting surface, such as the paper sheet, is so treated, it is passed through the varnish at a temperature not to exceed approximately 250 degrees F. and is held at that temperature for about 2 1/2 to 3 hours. These temperatures and the time of baking, the nature of the atmosphere in which baked, and the movement of that atmosphere will depend upon the supporting material. We merely mention typical examples.

45 50 The resulting product will have a wrinkled surface imitating leather, but the paper structure itself will not be disturbed except that on the

surface to which the product is applied there will be sufficient penetration to bond the coating to the paper. The surface will appear wrinkled and substantially without discoloration irrespective of its delicate colors. There will be provided a 5 smooth, heavy and wrinkled or pebbled surface which is a close imitation of genuine leather.

10 Varnish C and Varnish D can be varied in proportions of two to one of Varnish C to Varnish D, or two to one of Varnish D with respect to Varnish C. Raw China-wood oil can be varied in the same combination from one to ten parts. That is, from one to ten gallons, when gallons are used as the measure of the parts. The more China-wood oil used, the less the luster, and the 15 finer the finish or grain of the leather.

Different colors may be employed, such as: ultramarine blues; chrome yellows and greens; chromium oxide greens; toluidine and lithol reds, etc.

20 25 In the foregoing varnishes the proportions may be varied, but we prefer the proportions indicated, which we have found to be practical varnishes for this purpose.

By "cellulose backing" is comprehended a 25 variety of products, such as paper, pasteboard, cellophane and any others made of cellulose or its derivatives. Enumeration of these specific articles is not to be construed as a limitation or an exclusion of others of similar character.

30 35 It will be understood that we desire to comprehend within our invention such modifications as come within the scope of our claims and our invention.

Having thus fully described our invention, what 35 we claim as new and desire to secure by Letters Patent, is:

40 45 In a method of making imitation leather which comprises applying to one side only of flexible cellulose material a composition containing rosin modified phenol-formaldehyde resin, raw China-wood oil, cobalt linoleate, lead linoleate, a thinner and a coloring agent, and drying the coating at a temperature sufficiently high to form a wrinkled leather-like surface bonded to the flexible material by a partial penetration thereof, the temperature of drying not being carried to a point where the flexible cellulose material will be injured.

50 HARVEY G. KITTREDGE. ALBERT J. TURNER.